

Feb. 17, 1970

C. J. BENNING

3,496,063

ELECTROGRAPHIC REPRODUCTION ARTICLE AND METHOD

Filed Feb. 15, 1966

Fig. 1



Fig. 2



Calvin J. Benning

INVENTOR

BY

*Richard P. Plunkett*

ATTORNEY

# United States Patent Office

3,496,063

Patented Feb. 17, 1970

1

3,496,063

## ELECTROGRAPHIC REPRODUCTION ARTICLE AND METHOD

Calvin J. Benning, Clarksville, Md., assignor to W. R. Grace & Co., New York, N.Y., a corporation of Connecticut

Filed Feb. 15, 1966, Ser. No. 538,118  
Int. Cl. B32b 27/30, 27/32

U.S. Cl. 161—247

7 Claims

### ABSTRACT OF THE DISCLOSURE

Reproducing media for electrographic and high-speed electric printing substantially unaffected by humidity are made by milling polyethylene having a standard load melt index of substantially zero, and a density lying between 0.93 and 0.96, with photo-sensitive zinc oxide on the one hand for electrographic printing and carbon black on the other hand for high-speed electric printing. The zinc oxide film is laminated to a substrate of identical resinous composition but containing an electrically inert filler, whereas for high-speed electric printing a masking coat of identical resinous composition but containing a white pigment covers the black substrate.

This invention relates to media upon which images may be reproduced by high-speed electric printers and by electrostatic printing machines.

In an electric printer, the image is formed by an electrical discharge which passes to ground through a bi-color laminated sheet. The discharge burns through or melts away the top layer and exposes the underlying lamination, leaving usually, a black image appearing against a contrasting background.

In electrographic printing, on the other hand, a photo-sensitive material is incorporated in a coating which is spread upon a paper substrate. It is characteristic of certain materials, notably zinc oxide, that they will accept and retain an electric charge placed on their surface in the dark, but that when exposed to light, the electric charge will be dissipated in all exposed areas. Accordingly, if a sheet coated with, i.e. zinc oxide, is first charged and then is exposed through an original, the background loses its charge.

As applied to printing, the charged areas will attract and hold fusible ink particles which either may be brushed or flooded across the surface of the exposed sheet. When the sheet then is heated, the ink clinging to the charged area fuses to the substrate leaving a clear background area on which permanent printed characters appear in contrasting color.

One of the difficulties associated with high-speed electric printing is the control of the through-resistance. In media used in electrographic printers a characteristic difficulty is poor reproduction whenever the media has been exposed to varying humidities before its use. The amount of moisture contained in the substrate materially affects the color and definition of the reproduced image. Ideal storage conditions rarely are found in practice, for offices using such reproducing machines must store the reproducing media in any available space.

2

I have discovered that certain compositions containing either a conductive or a photo-sensitive substance may be produced as uniform surface sheets or films which are uniformly electrically responsive, and that such films are well adapted to form either the surface or the substrate layers of copy sheets for electric printing. I have found, too, that the sheets may be combined to produce composite sheets in a variety of combinations to adapt the sheets for use in the numerous models both of high-speed electric and electrographic printers.

The invention includes all-plastic laminated sheets or sheets in which the electrically responsive plastic compositions are combined either with a conductive or non-conductive paper layer. In all forms the invention presents two main aspects: (a) a substrate for high-speed electric printing in which the through-resistance may be accurately controlled, and (b) a composite sheet which is comparatively insensitive to change in humidity.

In the case of conductive substrates, not only may the initial through-resistance be controlled within reasonable limits, but by subsequent treatment, the resistance may be adjusted to precise values.

In the case of photo-sensitive media, a reproducing surface with lower sensitivity to humidity change may be laminated or spread on a variety of substrates. Several of the many possible combinations of surface and substrate will be set forth in separate examples.

Briefly stated, the present invention comprises a composite copy sheet adapted for use in electric printing apparatus comprising a substrate layer and a coating layer, at least one of said layers being electrically responsive and at least one of said layers being composed essentially of an intimate mixture of high density polyethylene having a standard load melt index of substantially zero, a particulate filler, and a plasticizer.

FIG. 1 illustrates a small cut sample of a sheet suitable for electrographic printing, and

FIG. 2 is a small sample of a sheet suitable for high-speed electric printing. For clarity, the thickness of the individual layers in the sheets has been greatly exaggerated.

The polyethylene used in the present invention should have a standard load melt index of substantially 0 and a high density, i.e. about 0.93 to 0.96.

The filler component of the instant composition, i.e. that comprised of the polyethylene, filler and plasticizer, may be electrically responsive or electrically non-responsive. The electrically responsive filler should be present in sufficient proportion to impart electrically responsive characteristics to the said sheet. Satisfactory results are produced from electrically responsive compositions comprised of about 15 to 30% of high density polyethylene of standard load melt index of substantially 0, 20 to 75% electrically responsive filler, and 10 to 50% plasticizer.

Representative of the electrically responsive fillers are photo-sensitive zinc oxide and conductive carbon black.

The standard load melt index (SLMI) used herein indicates the rate of extrusion of the polyethylene as measured under the conditions specified in ASTMD 1238-57T (Condition E). Since a high molecular weight polyolefin is more difficult to extrude than a low molecular weight

polyolefin, a standard load melt index of 0 would indicate a very high molecular weight polyolefin.

The high load melt index (HLMI) was measured as specified in ASTMD 1238-57T (Condition F).

Density was measured according to ASTMD 1505-57T.

All parts and percentages used herein are by weight unless otherwise specified.

#### EXAMPLE I.—PREPARATION OF SUBSTRATE

| Material       | Polymer                                                                                                         | Filler                                | Plasticizer                                       | Lubricant      |
|----------------|-----------------------------------------------------------------------------------------------------------------|---------------------------------------|---------------------------------------------------|----------------|
|                | Polyethylene having a standard load melt index of 0, a high load melt index of 1.4, and a density of 0.95-0.96. | Kaolin (Kaofil, avg. dia. <5 micron). | Petroleum oil (Shellflex 411,547 SSU at 100° F.). | Zinc stearate. |
| Pts. by weight | 28                                                                                                              | 54                                    | 26                                                | 1.             |

The substances were thoroughly blended and then worked at 400° F. in a "B" Banbury mixer for 6 minutes. The molten mixture was transferred to a 2-roll mill operating at 350° F., and sheeted out. The sheet, when cooled, was ground and pelletized by passing it through a 1" plastic extruder having a length to diameter barrel ratio of 24/1 and the screw having a compression ratio of 3/1 and operating at 325° F. at 50 r.p.m., at an extrusion pressure of 550 p.s.i. The pellets were dried and then fed through a tubing extruder having a 2" diameter die, operating with a 30 mil gap. Extrusion temperature was 350° F., screw speed, 60 r.p.m. The material passed through a 3 screen pack of 40-60-40 mesh at pressures of 1500 lbs. The hot tubing was blown to film thickness by the conventional "inflation" process. Air pressure within the trapped bubble was 0.5" water. Blow point was set at 10" above the die. Take-off speed of film was 100" per minute. Film thicknesses of from 1/2 to 2 mils were blown. The film was slit and rolled on cores.

The electrical resistivity of the photo-conductive surface was greater than  $3.88 \times 10^{-5}$  mho.-cm.<sup>-1</sup>. Since the laminate was comprised of a substrate of plastic composition relatively insensitive to water, and the photo-sensitive layer included photo-sensitive zinc oxide thoroughly embedded in plastic, it was found to withstand a wider range of humidity in the ambient atmosphere and yet

#### EXAMPLE II.—PREPARATION OF PHOTO-SENSITIVE LAYER

| Material       | Polymer                                                                                                         | Photo-sensitive material                                      | Plasticizer                                       | Lubricant      |
|----------------|-----------------------------------------------------------------------------------------------------------------|---------------------------------------------------------------|---------------------------------------------------|----------------|
|                | Polyethylene having a standard load melt index of 0, a high load melt index of 1.24 and a density of 0.94-0.95. | Photo-sensitive zinc oxide (Photox 801, avg. dia. <2 micron). | Petroleum oil (Shellflex 411,547 SSU at 100° F.). | Zinc stearate. |
| Pts. by weight | 16.5                                                                                                            | 71.5                                                          | 12                                                | 1.             |

<sup>1</sup> Total: 101.

The materials were blended in a ribbon mixer and then worked in a "B" Banbury for 6 minutes at 400° F. The molten "slug" from the Banbury was sheeted out on a 2-roll mill, operating at 350° F. The sheeted product was ground and converted into pellets as in the pelletizing step of Example I. The pellets were then fed through a tubing extruder and converted to film under the same conditions as in the film-forming step of Example I. The film was slit and rolled on cores.

#### EXAMPLE III

##### Production of laminate

The substrate film of Example I and the photo-sensitive film of Example II were cut into sheets and then placed between films of Mylar or aluminum foil and laminated by pressing the sheets for 4 minutes in a platen press heated to 165° C. Good lamination was secured

produce a better image than did photo-sensitive coatings on a paper base. The dielectric strength of the polyethylene used as a matrix for the photo-sensitive zinc oxide is high and amply sufficient to permit the laminate to accept and hold the electrostatic charge for more than 30 seconds in darkness. The charge dissipation factor is rapid, and total dissipation will occur within half a second when the surface is exposed to light through an ordinary paper original.

Other materials beside kaolin have proved equally satisfactory as fillers for the substrate, e.g., a composition containing 20% of the polymer of Example I, 54% of precipitated calcium carbonate, and 26% of the plasticizing oil, process as in Example I, performed substantially identically. A substrate formed of 15% of the polymer of Example I, 57% of milled and finely pulverized vermiculite, and 28% of the plasticizing oil, was equally satisfactory. The results were equally satisfactory when

aluminum silicates and powdered silica gels were used as fillers.

#### EXAMPLE IV

An electrosensitive film produced in accord with Example II was laminated to a sheet of 22 lb. "bread-wrap" paper approximately .0015" thick. The paper and photo-sensitive film were pressed in a platen press between 50 sheets of aluminum foil at 160° C. for 4 minutes. Good lamination on the paper substrate was secured when the photo-sensitive film thickness was from 1/2-1 mil. Reproductions on the paper-plastic laminate were substantially as good as on the all-plastic laminate, but the medium was somewhat more sensitive to varying atmospheric humidity. If the machine requires electrical conductivity in the substrate, paper containing a conductive filler, e.g., carbon black, may be substituted for the substrate.

#### EXAMPLE V.—PRODUCTION OF CONDUCTIVE SUBSTRATE

| Material       | Polymer                                                                                                         | Conductive material                                         | Plasticizer                                       | Lubricant      |
|----------------|-----------------------------------------------------------------------------------------------------------------|-------------------------------------------------------------|---------------------------------------------------|----------------|
|                | Polyethylene having a standard load melt index of 0, a high load melt index of 1.24 and a density of 0.94-0.95. | Carbon black (Vulcan XC72, Cabot Co., avg. dia. <1 micron). | Petroleum oil (Shellflex 411,547 SSU at 100° F.). | Zinc stearate. |
| Pts. by weight | 29.8                                                                                                            | 22.5                                                        | 48.7                                              | 1.             |

when substantially uniform substrate films and photo-sensitive films were each from 1/2-1 1/2 thousandths inch thickness.

The materials were blended and mixed in a "B" Banbury at 400° F. for 6 minutes. The Banbury batch was transferred to a 2-roll mill operating at 350° F. and sheeted

out. Subsequently, the sheet was ground and pelletized on a 1" thermoplastic extruder having a length to diameter barrel ratio of 24/1 and a compression ratio of 3/1 on the screw, and operating at 50 r.p.m. at 325° F.; extrusion pressures were 550 p.s.i. The pellets were dried and fed into a 1" 24:1 film extruder equipped with a 2" diameter film die having a 30 mil gap. Extrusion pressure was 1500 p.s.i., temperature 350° F., screw speed 60 r.p.m. A screen pack of 40-60-40 mesh was used. The material was reduced to film thickness by the conventional bubble method at a bubble pressure of 0.5" of water. The take-off speed was 100" per minute when films of 1-2 mil thicknesses were blown. The film was slit and rolled on cores.

In electric discharge (high-speed) printing, the through-resistance of the substrate should be as low as possible. Very low resistance values may be secured by extracting the plasticizer with a light petroleum solvent. The time of extraction (a few seconds only) may be controlled to produce precise low resistance values.

#### EXAMPLE VI

Sheets of the material of Example V were soaked briefly in a light petroleum solvent to extract the plasticizer. Extraction of the plasticizer for 1 second in "Solvesso" No. 1 reduced the through-resistance of a 1-mil film to approximately 5 ohms. At the same time, extraction conditioned the conductive film to receive and hold the masking coat.

#### EXAMPLE VII.—PREPARATION OF THE MASKING COAT

|          | Resin         | Filler         | Whitener                                               | Solvent            |
|----------|---------------|----------------|--------------------------------------------------------|--------------------|
| Material | White shellac | Georgia kaolin | Titanium dioxide<br>(DuPont Titanox<br>pigment grade). | Denatured alcohol. |

A sheet prepared according to Examples V and VI was anchored on the bed of a knife-coater and the above mixture, after being thoroughly stirred and blended, was spread on the substrate to a film thickness of .00025. The coating was allowed to dry.

The dry laminate was tested in a high-speed electric printer. The white coating burned away in the areas subject to discharge, leaving a clear black image. Alternate formulations for the coating which gave substantially equal results in electric discharge printing were composed of bentonite 20 parts, and 5 parts of a whitener (titanium dioxide) suspended in 60 parts of a low molecular weight acrylic resin solution. Both roll and knife coating of the above formulae produced substantially equal results.

#### EXAMPLE VIII.—PREPARATION OF THE MASKING LAYER

|                | Polymer                                                                                                                          | Filler                                                               | Plasticizer                                                                                         | Whitener                                               |
|----------------|----------------------------------------------------------------------------------------------------------------------------------|----------------------------------------------------------------------|-----------------------------------------------------------------------------------------------------|--------------------------------------------------------|
| Material       | Polyethylene<br>having a standard<br>load melt index of<br>0, a high load<br>melt index of 1.4<br>and a density of<br>0.95-0.96. | Calcium carbonate<br>particle size .1-<br>.3 microns<br>(Purecal 0). | Petroleum oil<br>boiling point<br>greater than<br>300° C. (Shellflex<br>411 547 SSU at<br>100° F.). | Titanium dioxide<br>(DuPont Titanox<br>pigment grade). |
| Pts. by weight | 20                                                                                                                               | 65                                                                   | 15                                                                                                  | 5                                                      |

The materials were blended and converted into films following procedures given in Examples I and II.

A laminate was made by sandwiching sheets made according to Examples V and VI, 1/2 mil in thickness, and sheets from Example VIII, 1 mil in thickness, between sheets of highly polished Ferrotype Sheets and pressing the sandwich in a platen press for 4 minutes at 160° C. The resulting laminates were tested on a high-speed electric printer, and clear, sharply outlined black images were produced.

Although it is not strictly necessary, the addition of a lubricant in the amount of 1% to blends of polyethylene and filler given in Examples I, II, V and VIII improves the extrusion characteristics of the blend. A 1 weight percent addition of zinc stearate is recommended.

#### EXAMPLE IX

A sheet as made by Example II, 1 mil in thickness, was adhesively joined to a 22-lb. bread-wrap paper substrate which, prior to lamination, had been coated with a spread coat of vinylidene chloride copolymer (Daran Emulsion). The photo-sensitive film was pressed against the paper by passing the same through a set of rubber-covered squeeze rolls. The reproduction results were substantially the same as those reported in connection with Example IV.

A photo-sensitive coating can, with advantage, be spread on a substrate made according to Example I or on one containing any suitable inert filler. Lower hydroscopic sensitivity as compared to a paper based sheet will be obtained.

#### EXAMPLE X

A sheet prepared according to Example I was extracted by soaking the sheet for 45 seconds in Solvesso #1. The sheet was then dried and subsequently was spread-coated with the following thoroughly-blended mixture.

|                                                                                 | Weight percent |
|---------------------------------------------------------------------------------|----------------|
| Material—Photo-sensitive zinc oxide                                             | 83             |
| Vehicle—Vinyl acetate emulsion (Everflex G) Dewey<br>& Almy Div. of W. R. Grace | 17             |

The sheets were dried and then tested in an S.C.M. copier. Good reproduction was achieved. Anchorage of the

spread film was excellent when the plasticizer extraction step was used.

As a general statement, the photo-sensitive zinc oxide should constitute as high a proportion as possible of the total mass of the photo-sensitive layer. Operative results will be obtained when the weight proportion of the zinc oxide in the total mixture exceeds 60% and preferably is in the approximate range of 70%.

The electrically conductive layers containing carbon black should also have as high a proportion of conductive black to polyethylene as is possible, and operative results will be secured when the weight proportion of carbon black to the total mixture exceeds 20%, and preferably approximately 29%.

The above results cannot be obtained from low-density polyethylene since compositions containing the requisite amount of filler material, e.g. zinc oxide or carbon black, then are brittle and difficult to work. When, however, the molecular weight of the polyethylene is in excess of 500,000 and the standard load melt index is substantially 0, workability of the mixture is possible when it is plasticized and the high molecular weight imparts sufficient strength, even at the high degree of filler loading necessary, to allow the material to be sheeted out and subsequently handled.

Of the very wide range of plasticizers which permit processibility at these high percentage loadings, any of those such as dibutyl sebacate, asphalt, and others which are electrically inert, are suitable. However, the very low

cost, excellent electrical characteristics, and easy extractability make petroleum oils especially suited as plasticizers in this invention.

The zinc oxide should be photo-sensitive, and preferably should be sensitized to light in the visible spectrum in known manner by the addition of minor proportions of sensitizing dye. Such zinc oxides are commercially available.

The term "electrically responsive" as used in this specification and the appended claims is intended to apply to filling materials which are themselves electric conductors such as, e.g., conductive carbon black and substances which accept and hold an electric charge, such as, e.g. photo-sensitive zinc oxide.

When the plasticizer is present, the through-resistance of the combination may be too high to permit use in certain high-speed electric printers, but, as has been described, the resistance can be dropped to very low and predetermined levels by extraction of the plasticizer. Operative through-resistances should be less than 20 ohms, and preferably about 5 ohms. The surface resistance should be less than 2500 ohms. Extraction of the plasticizer has the added advantage that the anchoring of the top coat or top lamination to the substrate is greatly improved.

In instances where a photo-sensitive coat is anchored to a paper substrate, an adhesive bond may be utilized. The adhesive may be rubber cement, polyvinyl acetate, casein, or the like, which is spread on the paper prior to laminating the photo-sensitive coating to the paper substrate. Generally speaking, a wide range of adhesives, provided they are not insulators, and have a through-resistance not in excess of 20 ohms, in the adhesive layer will be found to be practical.

It will be appreciated from the above examples that other methods of joining the two layers may be utilized, e.g. a conductive base coat may be led past the orifice of a slit extruder and the non-conductive white coat may be combined with a conductive substrate by passing the combination between squeeze rolls. A laminated, all-plastic sheet may be made by combining the products of two slit extrusions—one photosensitive and one insensitive. Such changes will readily suggest themselves to one who is familiar with laminating and extrusion techniques and the content of this disclosure.

What is claimed is:

1. Composite copy sheet adapted for use in electric printing apparatus comprising a substrate layer and a coating layer, both of said layers being formed from the milled and sheeted mixture of (a) from 15-30% by weight of an ethylene polymer having a standard load melt index of zero, and a density lying between 0.93 and 0.96, and (b) from 20-75% weight percent of a particulate filler, the said filling material in at least one of said layers being a particulate electrically responsive filler substance selected from the class consisting of carbon black and photo-sensing zinc oxide.

2. Composite copy sheet as claimed in claim 1, adapted for use in electrographic printing apparatus comprising a substrate layer composed of the said ethylene polymer and filling material selected from the class of fillers consisting of kaolin, pulverized vermiculite, aluminum silicate, and powdered silica gel, and wherein the upper layer com-

prises a mixture including the said resin and photo-sensitive zinc oxide.

3. Copy sheet as claimed in claim 2 wherein the proportion of zinc oxide in the top lamination is about 71%.

4. Copy sheet as claimed in claim 1 wherein the substrate layer is formed of the said resinous composition and approximately 22½% of carbon black and wherein the said top layer is a masking coat comprising the said resinous composition and a white pigment.

5. The process of preparing image sheets suitable for use in electrographic reproduction apparatus which comprises milling from 15-30 parts by weight of an ethylene polymer having a standard load melt index of zero, and a density lying between 0.93 and 0.96, and from 20-75 parts by weight of photo sensitive zinc oxide, and from 10-50 parts by weight of a plasticizer, forming the milled mixture into sheets, preparing a second composition containing the said resin in proportions of from 15-30 parts by weight, and from 20-75 parts by weight of a filler selected from the class of filling substances consisting of kaolin, calcium carbonate, pulverized vermiculite, aluminum silica, and silica gel, and from 10-50 parts by weight of a plasticizer, forming the said composition into a sheet and laminating the first and the second named sheets together by heat and pressure to form the photo-sensitive reproduction medium.

6. The process of preparing image sheets suitable for use in electric printer apparatus which comprises forming a sheet of from 15-30 parts by weight of an ethylene polymer having a standard load melt index of zero, and a density lying between 0.93 and 0.96, and from 20-75 parts by weight of a white pigment comprising calcium carbonate and titanium dioxide, forming a second named sheet from the said resin and from 20-29% of electrically conductive carbon black and a plasticizer, and laminating the first and second named sheets together by heat and pressure to form an image sheet suitable for high-speed electric printing.

7. That process of adjusting the through electrical resistance of image sheets produced according to claim 6, which includes extracting the plasticizer from the said second named sheet with a petroleum solvent prior to laminating the first and second sheets together, whereby the through resistance of the second sheet is reduced to values of less than 20 ohms.

#### References Cited

##### UNITED STATES PATENTS

50 3,010,884 11/1961 Johnson et al. \_\_\_\_ 117—201 X  
3,245,833 4/1966 Trevoy \_\_\_\_\_ 117—201

##### FOREIGN PATENTS

55 949,605 2/1964 Great Britain.  
964,829 7/1964 Great Britain.

WILLIAM L. JARVIS, Primary Examiner

U.S. CL. X.R.

60 96—1; 117—63, 201; 156—182, 242; 161—410; 204—2;  
264—105